

Aug. 14, 1956

L. THORINGTON

2,759,119

COMBINATION LIGHT SOURCE

Filed Sept. 16, 1953

2 Sheets-Sheet 1

FIG. 1.



FIG. 2.



FIG. 4.

FIG. 3.



INVENTOR.  
LUCE THORINGTON.

BY

*John J. Kelly*

ATTORNEY.

Aug. 14, 1956

L. THORINGTON

2,759,119

COMBINATION LIGHT SOURCE

Filed Sept. 16, 1953

2 Sheets-Sheet 2

FIG. 5.



FIG. 6.



FIG. 8.



FIG. 7.



INVENTOR.  
LUKE THORINGTON

BY  
  
ATTORNEY.

# United States Patent Office

2,759,119

Patented Aug. 14, 1956

1

2,759,119

## COMBINATION LIGHT SOURCE

Luke Thorington, Glen Gardner, N. J., assignor to Westinghouse Electric Corporation, East Pittsburgh, Pa., a corporation of Pennsylvania

Application September 16, 1953, Serial No. 380,408

4 Claims. (Cl. 313—109)

This application is a continuation-in-part of my application Serial No. 55,672, filed October 21, 1948, now abandoned, and my application Serial No. 126,506, filed Nov. 10, 1949.

This invention relates to the color modification of light sources, especially incandescent electric lamps, and to the phosphors used in effecting this modification.

The principal object of my invention, generally considered, is to make use of the electron emission, as well as the ultra-violet radiation, from the filament of an incandescent electric lamp to act on a phosphor coating on the inner surface of the envelope of such a lamp, in order to produce a worthwhile part of the emitted light by photoluminescence or low-voltage high-current high-temperature cathodoluminescence with or without gas discharge phenomena.

Another object of my invention is to make use of the electron-emission from the filament of an incandescent electric lamp to, even at line voltage, excite an efficient high temperature phosphor to thereby improve the light source in color and efficiency.

A further object of my invention is to produce an incandescent electric lamp containing a coating of phosphor on an inner conductive surface on the envelope thereof, to which coating one side of the power line is connected, the midpoint of the filament is connected thereto, or a direct-current is applied between the filament and the coating, to cause electrons emitted by the filament to move toward and impinge on the phosphor carried on the inner surface of the envelope.

A still further object of my invention is a lamp, such as described in the preceding paragraph, in which a conductive phosphor coating is substituted for the conductive surface coating carrying the phosphor.

An additional object of my invention is to employ manganese-activated zinc fluoride as a coating on the inner surface of the envelope of an incandescent electric lamp, to add bright green cathodoluminescence at elevated temperatures to the lamp output, to thereby not only improve the efficiency but modify the color of the light output of said lamp.

Another object of my invention is to substitute for the normal tungsten filament of an incandescent lamp, of the character above described, a selective radiator such as a Welsbach mixture or Nernst glower in a quartz bulb.

A further object of my invention is to add gas or vapor to a cathodoluminescent lamp, such as above described, to provide a versatile light source in which gas discharge phenomena may contribute to the output, in addition to the other sources of illumination.

Other objects and advantages of the invention will become apparent as the description proceeds.

Figure 1 is a graph comparing the energy distribution of a tungsten filament lamp with that weighted by the eye sensibility function.

Figure 2 is an elevational view, with parts in axial section, of an incandescent filament lamp embodying my invention.

2

Figure 3 is a view corresponding to Figure 2, but showing an incandescent filament lamp of the reflector type.

Figure 4 is a view corresponding to Figure 2, but showing a modification in which the coating on the inner surface of the envelope is connected to one end of the filament.

Figure 5 is a view corresponding to Figure 4, but showing a modification in which the coating is connected to the mid-point of the filament.

Figures 6 and 7 are views corresponding to Fig. 4, but showing modifications in which a direct potential is applied between the midpoint and one end of the filament, respectively, and the phosphor coating, in order to uniformly direct the emitted electrons from the filament to said coating.

Figure 8 is a view corresponding to Fig. 4, but showing a substitution of an electron emitter in an inner quartz or refractory translucent bulb which is, in turn, enclosed in an outer bulb.

In the present case I am proposing a new lamp, that is, a combination incandescent and cathodoluminescent lamp which may also be augmented by gas discharge phenomena or photoluminescence.

Most of the energy input of an incandescent light source is wasted as heat, a very difficult form of energy to reconvert efficiently into luminous energy. However, incandescent bodies also produce electrons by thermionic emission. We have here, what is ordinarily unused in our incandescent electric lamps, something for which we spend great amounts of energy to obtain in electronic devices such as vacuum tubes, discharge lamps, and television tubes. I propose to make use of this electron emission at ordinary line voltages of 110 to 440 volts, to excite an efficient high-temperature phosphor, and so considerably improve the light source as a whole, that is, both in color and efficiency.

One method of accomplishing the results desired is to first produce a conductive surface on the inside of the lamp envelope. This may be done by using any one of the several transparent conductive coatings which are now available. A cathodoluminescent phosphor which functions at low voltages, and at the operating temperature of the bulb or envelope, is then coated over the conducting layer. In one mode of operation, one side of the filament is connected to the conductive coating or the latter may be connected to the midpoint of the filament, and in still another the midpoint or other portion of the filament has a separate unidirectional potential applied thereto. In any case, electrons thermally ejected from the filament are accelerated toward the phosphor where they impinge and cause the coating to luminesce. It is also desirable that the coating luminesce under impingement thereon by the ultra-violet radiations generated in the envelope by the filament or other source.

Another mode of accomplishing the desired end is to coat the inside of the envelope with a phosphor which is electrically conductive and connect it as above, first eliminating the separate transparent conductive coating.

In each case the phosphor desirably functions at high temperatures and transmits visible radiations. The following are considered the most desirable properties of a phosphor for the application here disclosed.

1. The phosphor should respond to relatively low voltage, high current cathode ray excitation.
2. It should function at relatively high temperatures.
3. It should efficiently transmit visible radiation.
4. It should be electrically conductive.
5. It should luminesce in the most visually efficient portion of the spectrum, that is, the green.

I discovered that the ordinary orange cathodoluminescence of  $ZnF_2:Mn$ , while being quenched at elevated temperatures, does at even higher temperatures emit a

bright green cathodoluminescence. This phosphor fulfills all the above requirements and, in addition, can be easily evaporated and condensed as a thin clear film. A lamp embodying this phosphor is somewhat analogous to the color-corrected mercury lamp of the parent application, Ser. No. 126,506, previously referred to. That is, it has a phosphor maintained at or near its optimum light-generating temperature.

The lamp of this disclosure, however, is also not necessarily limited to phosphors having peak efficiency at elevated temperatures. Neither is it limited to incandescent lamps of the common variety. For example, it may be desirable to combine an incandescent selective radiator, such as a Welsbach mixture or Nernst glower, with a phosphor-coated bulb. It is considered desirable to use a quartz or other high-temperature bulb, for operation of the phosphor coating at temperatures higher than attainable with ordinary bulbs.

The possibilities of such a source are extremely interesting. The highest luminous efficiencies reported thus far for the cathodoluminescence process are in the neighborhood of 90 lumens per watt. This is for high voltage excitation of sulfide type phosphors. However, with the proper phosphor there is no fundamental reason why high efficiency cannot be attained with low voltage excitation. It is possible to draw emission currents of about  $\frac{1}{2}$  ampere from an ordinary 100 watt general service lamp filament. For a potential difference of 100 volts, this would mean 50 watts of available power for conversion into light by cathodoluminescence. For a phosphor of 50 lumens/watt cathodoluminescence efficiency, this would mean 2500 lumens additional light, that is, more than twice the amount of light generated by the filament itself when operating in vacuum.

The efficiency of a tungsten filament in vacuum is about 10 lumens/watt, when all interdependent factors are adjusted to the optimum. The combination efficiency would thus be near 23 lumens per watt, or considerably higher than the gas-filled incandescent lamps and the color would be improved. Assuming higher efficiencies attainable in the phosphor, we may conceivably reach 40 lumens per watt for such a lamp.

Most cathodoluminescent materials are known to have an effectively "dead" layer surrounding the individual phosphor crystals. Thus in order to actually transfer energy to the active centers of the crystals the electrons must first traverse the "dead" layer. In so doing, they lose a large part of their energy for which no luminescence is emitted. Thus, the electrons must be given sufficient energy before impact to not only traverse this "dead" layer, but to also excite the active centers after traversing the dead layer. The ways in which electrons expend their energy in luminescent materials are as follows:

1. A part is lost as heat in the "dead" layer.
2. A part is lost in ejection of secondary electrons.
3. A part is used to engage the active centers and is

transformed and emitted as luminescence.

It is thus seen that a conducting phosphor having active centers on its surface may be activated by very low-energy electrons. Such a material is  $ZnF_2:Mn$ ; it is very conductive and may be excited by 10 volt electrons. In addition to a lamp such as above described in which the electron-emitting filament is in a vacuum, I may substitute for said vacuum a gas or vapor to produce a versatile light source embodying all of the methods of generating light heretofore found practical, except that used in photoflash lamps. In other words, with a gas-filled incandescent lamp, the envelope of which is phosphor-coated and connected as before described, I may attain light by not only:

#### 1. Incandescence

2. Luminescence, including both cathodo- and photo-luminescence, but also by
3. Gas discharge phenomena.

The lamp in its greatest simplicity may take the form of an ordinary incandescent lamp having an inside coating of conductive phosphor, such as manganese-activated zinc fluoride, electrically connected to one end, or an intermediate part, of the filament. A small amount of a suitable gas or vapor is introduced so that a discharge may be maintained between the filament and phosphor coating. The phosphor should be responsive to both the ultra-violet, if any, of the discharge, as well as to low voltage electrons. The mentioned phosphor is excited by ultra-violet radiations having wave-lengths shorter than 2200 A. U., by electrons with energies as low as 10 volts, and its green luminescence is stable at high temperatures.

The presence of a small amount of gas or vapor in the envelope also serves to increase the total of current available for the cathode-ray excitation of the phosphor. Current limitation of the discharge is effected by a separate series resistance, by the semi-conductive property of the phosphor coating itself, by a choke or by another ballasting device. Certain types of discharges are self-limiting. This property would be valuable in a lamp embodying my invention.

Advantages of the combination source would be similar to those previously disclosed for the incandescent-cathodoluminescent vacuum lamp, viz., it would operate in ordinary lamp sockets and would have considerably higher efficiency and better color than ordinary incandescent lamps.

Color and color rendition of the source could be varied widely by changing the phosphor, gas filling, or temperature of the filament. As in the incandescent-cathodoluminescent vacuum lamp, the incandescent body may preferably be a selective radiator such as thoria; 1% ceria, instead of a tungsten filament, and the bulb may preferably be of quartz or hard glass.

Referring to the drawing in detail, and first considering Figure 1, there is shown a curve (a) which represents the energy distribution of a tungsten filament lamp operating at a color temperature of 2854° K. which is the operating temperature of an ordinary 100 watt general service lamp. Curve (b) is the same distribution weighted by the eye sensibility function. Thus, if the total area under curve (a), between  $\lambda=4000$  A. U. and 7000 A. U., is proportional to the total visible radiated watts, then the area under curve (b) is proportional to the total lumens. Curve (c) is a plot of the eye sensibility function used in arriving at curve (b) and shows the relative "see-ability" of the various colors of light.

It is apparent that the extremely low efficiency of the tungsten filament light distribution below 5000 A. U. is due to the fact that the energy from the filament is decreasing rapidly in the range, and also the eye sensibility is decreasing even more rapidly. Of course, it is impossible to change the tungsten filament light distribution without changing its temperature and this is not desirable. However, the actual number of lumens produced by the tungsten radiation below 5000 A. U. can be varied by shifting this energy to more visibly efficient regions of the spectrum by the process of luminescence.

Considering a conventional 100 watt, A-21 gas-filled tungsten lamp, the following is true: color temperature=2854° K. Total lumens=1630 (initial)

Per cent of total radiation below 4000 A. U.=16.3%  
Per cent of total radiation below 7500 A. U.=10.81%  
Per cent of radiation in visible=10.65%  
Total emitted visible watts (4000-7500 A. U.)=10.65 watts

Total emitted u. v. watts (below 4000 A. U.)=.16 watts  
Thus the ordinary wasted portion of energy below 4000 A. U. for this lamp amounts to about 1.5% of that

emitted in the visible. If this energy could be transferred to visible, using a phosphor such as here disclosed, or possibly better still, a phosphor having an emission spectrum comparable with that of zinc silicate and a quantum efficiency as good, then an appreciable increase in lumens would result. For example,

|                                                |    |
|------------------------------------------------|----|
| Assume luminosity of fluorescence spectrum     | 8  |
| Assume quantum efficiency                      | 9  |
| Assume energy loss factor (3600 to 5300 A. U.) | 7  |
| Assume absorption loss factor                  | 95 |

Total theoretical lumens =  $16 \text{ watts} \times 680 \text{ lumens/watt} = 109 \text{ lumens}$ ;  $109 \text{ lumens} \times \text{spectrum luminosity} = .8 \times 109 = 87 \text{ lumens}$ ;  $87 \text{ lumens} \times \text{quantum eff.} = 73 \text{ lumens}$ ;  $73 \text{ lumens} \times \text{energy loss} = .7 \times 73 = 51 \text{ lumens}$ ;  $51 \text{ lumens} \times \text{absorption loss} = .95 \times 51 = 49 \text{ lumens}$ . Therefore, the total lumen gain = 49 lumens, and total lamp efficiency is

$$\frac{1630 + 49}{100} = 16.8 \text{ l. p. w.}$$

The increase in lumens would amount to about 3% and the overall color of the light would be improved over the bare tungsten filament.

Where highest lumens are desired, regardless of color, it is possible to improve the lumen efficiency by about 11% by utilizing all the radiation below 5070 A. U. to produce luminescence having higher luminosity. One tenth of the lumens of the lamp (163 lumens) under consideration are below 5070 A. U., but by using a phosphor over 350 lumens could be produced. The total lumens of the source would then be  $1630 + 350 - 163 = 1817$  lumens; the color would be yellowish but not displeasing because of the large excess of red already present. Phosphors for the above applications are available now, but the difficulty is that they are quite temperature-sensitive and, therefore, would necessitate the use of large cumbersome bulbs. The problem in this respect is the same as for the phosphor-coated HPMV lamp. I therefore, propose lamps such as illustrated in Figs. 1 to 4, inc., of the parent application Serial No. 126,506, previously referred to, but in which an incandescent filament lamp, having an ultra-violet-transmitting envelope, replaces the HPMV lamp.

In Fig. 2 there is shown an embodiment of my invention in which a phosphor coating  $34^d$  is applied directly to the inner surface of the envelope  $22^d$  of an incandescent electric lamp  $12^d$  adapted for alternating or direct-current operation. This lamp may be of otherwise conventional construction; involving a screw-threaded base  $21^d$ , a stem  $19^d$ , and an incandescent desirably coiled filament  $25^d$  supported on leads  $17^d$  and  $18^d$  extending therefrom. The filament may be braced by a spud  $15^d$ , the normally lower end of which is embedded in a button on the end of an arbor  $16^d$  extending from the stem  $19^d$ . The envelope  $22^d$  may be evacuated or contain an inert gas, as desired in accordance with conventional practice.

In this case, the ultra-violet light given off by the filament, when incandesced, acts on the phosphor coating  $34^d$ , resulting in the generation of fluorescent light which correspondingly augments and modifies the spectrum of the light given by the filament. The phosphor desirably has a green-yellow emission and is activated by long and short ultra-violet rays, and a quantum efficiency near .9 or above. Such phosphors as manganese-activated zinc orthogermanate and zinc-activated zinc oxide are examples of suitable phosphors for this application. However, manganese-activated zinc fluoride, although not excited by long ultra-violet rays, is particularly desirable as it operates efficiently at the relatively high temperature of the envelope of an incandescent lamp under electron excitation, thereby making it especially suitable for the applications of Figs. 4 to 8, incl.

Referring now to the embodiment of my invention illus-

trated in Fig. 3, there is shown a lamp  $12^e$ , also adapted for alternating or direct-current operation, which includes an incandescent filament  $25^e$ . The lamp  $12^e$  corresponds generally with the lamp  $12^d$  of the preceding embodiment, except that it has a larger and differently-shaped envelope  $22^e$ , and a portion thereof is coated with reflecting material  $35$ , such as silver or aluminum, to concentrate the light on the remainder of bowl  $36$  of the envelope, which is coated with fluorescent material  $34^e$ . The fluorescent material in this instance may correspond with that of the preceding embodiment, although because the envelope of this lamp may operate at a lower temperature, it need not be such that will operate efficiently at the relatively high temperature of the lamp of the preceding embodiment.

Referring now to the embodiment of my invention illustrated in Fig. 4, there is shown an incandescent electric lamp  $12^f$  to be used on alternating current only or on direct current in which the right hand end of the incandescent filament  $25^f$ , as viewed in said figure, is connected to the negative pole of the supply. It comprises an envelope  $22^f$ , based as indicated at  $21^f$  and enclosing a stem  $19^f$  supporting said filament. In the present instance, the filament  $25^f$  may be formed of tungsten, thoriated tungsten, or other material having high luminous efficiency and high electron-emissivity. The inner surface of the envelope desirably carries a conductive coating, to which is applied a film or coating of a photo-and cathodoluminescent phosphor. Such conductive coating is desirably a conductive glass or glaze containing tin oxide, examples being those designated by the Pittsburgh Plate Glass Co. trademark "Nesa," and the Corning Glass Works trademark "EC". As another example, a conductive tin and antimony compound which may be produced as described and claimed in the Mochel Patent No. 2,522,531, may be used. As an alternative the phosphor coating may be mixed with conductive material, if not naturally conducting.

The envelope may be either evacuated or contain inert or rare gas such as nitrogen, argon, neon, krypton, xenon, or mixtures of said gases. The pressure of the gas, if used, is desirably not high enough to allow a destructive arc discharge across the filament.

In order to create an electron flow between the filament and the phosphor during operation, one side of the filament is connected to the phosphor coating  $34^f$ , as by a resilient extension, indicated at  $37$ , from the lead  $18^f$ , so that during operation the phosphor coating is activated, not only by ultra-violet radiation, but also by an electron discharge thereto. If used on alternating current, the electron discharge will, of course, only pass to the coating  $34^f$  on alternate half cycles, that is, only when the filament  $25^f$  is negative with respect thereto.

Fig. 5 shows a lamp  $12^g$ , which may be identical with the lamp  $12^f$  of Fig. 4, except that it may be used on alternating or direct current without regard to polarity. In this case the phosphor coating  $34^g$  is connected to the midpoint  $38$  of the filament, as by means of supporting lead  $39$ , as indicated at  $37^g$ .

Fig. 6 represents a lamp  $12^h$ , which may be like the lamp  $12^f$  of Fig. 4, except that it is intended for use on only alternating current. The midpoint  $38^h$  of the filament  $25^h$  is connected to the negative side or pole of a battery  $39$ , or other source of unidirectional power, which here serves as the force causing electrons to flow to the phosphor coating  $34^h$ , as through the intermediate contact or ring  $41$  of a medium or mogul "3-lite" base  $21^h$ , which may in this case be used on the lamp instead of a conventional screw-threaded medium base. The positive pole of the source  $39$  is connected to the phosphor coating  $34^h$  on the inner surface of the envelope  $22^h$  as by a lead  $42$  through the envelope neck or in any other suitable manner.

Fig. 7 represents a lamp  $12^k$ , which is intended for use on only alternating current. It may be like the lamp  $12^f$

7 of Fig. 4 except that one end of the filament 25<sup>k</sup> is connected to the negative side or pole of the battery 39<sup>k</sup>, or other source of unidirectional power. Such connection may be through the shell of a medium or mogul "3-lite" base 21<sup>k</sup>, which may in this case be used on the lamp instead of a conventional screw-threaded base. The positive pole of the source 39<sup>k</sup> is connected to the phosphor coating 34<sup>k</sup> on the inner surface of the envelope 22<sup>k</sup>, as by an auxiliary lead 42<sup>k</sup> from the intermediate contact or ring 41<sup>k</sup> of said base, and a resilient contact member 37<sup>k</sup> extending from said auxiliary lead. This means that during operation of the lamp, electrons are drawn from the filament 25<sup>k</sup> to the phosphor coating 34<sup>k</sup>, as in the embodiment of Fig. 6. The only essential difference is that the unidirectional potential is applied between one end, rather than the central portion, of the filament and the phosphor coating.

In the embodiment of Fig. 8, a lamp 12<sup>m</sup> is represented which is intended for use on alternating current or on direct current in which the top end to the electron-emitter 25<sup>m</sup>, as viewed in said figure, is connected to the negative pole of the supply. It may be like the lamp 12<sup>f</sup> of Fig. 4 except that the filamentary light source is here replaced by the electron-emitter 25<sup>m</sup> enclosed in an inner quartz bulb 43, or other high-temperature translucent inner envelope, which may be either evacuated or contain low-pressure fill gas, like the envelope 22<sup>f</sup> of Fig. 4. The quartz bulb 43 is supported by the leads 17<sup>m</sup> and 18<sup>m</sup> extending from the stem 19<sup>m</sup> or in other suitable manner in an outer envelope 22<sup>m</sup> which outer envelope may be clear of a phosphor coating, and such a coating applied to the inner surface of the quartz envelope 43, as indicated at 34<sup>m</sup>. However, if desired, the outer envelope 22<sup>m</sup> may carry the phosphor coating, and the inner envelope be clear, if cathodoluminescence is to be sacrificed. If the coating is applied to the inner envelope, there is a contact between it and one side of the electron emitter 25<sup>m</sup>, as indicated at 37<sup>m</sup>.

The size of the phosphor-carrying envelope is, in each embodiment, desirably such that during operation it is maintained at a temperature approximately optimum for the generation of visible light by the phosphor coating. However, such temperature may range between one approximately optimum and one higher or lower to allow for selection of a convenient bulb, that is, avoid undesirably large or small envelope size.

Although preferred embodiments have been disclosed, it will be understood that modifications may be made within the spirit and scope of the invention.

I claim:

1. In combination, a power-operable incandescent source of radiant energy including ultraviolet radiations and electrons, a light-transmitting envelope surrounding said source, a light-transmitting coating on the inner surface of said envelope comprising a phosphor-including electrically-conductive coating having an efficient output at the normal envelope operating temperatures and for which production of light in the green region of the spectrum is high upon impingement of said coating by radiant energy and electrons emanated from said source when operated, means electrically connecting said coating to said source, said source when operated producing visible radiations amounting to a substantial portion of the total visible radiations produced by said source and said phosphor, whereby the visible light from said source is augmented and the color thereof modified by the light generated by said phosphor.

5 2. In combination, a power-operable incandescent source of radiant energy including ultraviolet radiations and electrons, a light-transmitting envelope surrounding said source, a light-transmitting coating on the inner surface of said envelope comprising a phosphor-including electrically-conductive coating having an efficient output 10 at the normal envelope operating temperatures and for which production of light in the green region of the spectrum is high upon impingement of said coating by radiant energy and electrons emanated from said source when operated, means for applying a potential between said coating and said source so that electrons emitted by said source during operation will be drawn to said coating, said source when operated producing visible radiations amounting to 15 a substantial portion of the total visible radiations produced by said source and said phosphor, whereby the visible light from said source is augmented and the color thereof modified by the light generated by said phosphor.

3. In combination, a power-operable incandescent 20 source of radiant energy including ultraviolet radiations and electrons, a light-transmitting envelope surrounding said source, a light-transmitting coating on the inner surface of said envelope comprising a phosphor-including electrically-conductive coating for which production of 25 light in the green region of the spectrum at the normal envelope operating temperatures is high upon impingement of said coating by radiant energy and electrons emanated from said source when operated, said phosphor being one of the group consisting of manganese-activated zinc fluoride, manganese-activated zinc orthogermanate, and zinc-activated zinc oxide, means electrically connecting said coating to said source, said source when operated producing visible radiations amounting to a substantial portion of the total visible radiations produced by 30 said source and said phosphor, whereby the visible light from said source is augmented and the color thereof modified by the light generated by said phosphor.

4. In combination, a power-operable incandescent 40 source of radiant energy including ultraviolet radiations and electrons, a light-transmitting envelope surrounding said source, a light-transmitting coating on the inner surface of said envelope comprising a phosphor-including electrically-conductive coating having an efficient output 45 at elevated temperatures and for which production of light in the green region of the spectrum at the normal envelope operating temperatures is high upon impingement of said coating by radiant energy and electrons emanated from said source when operated, the size of said envelope being such that during operation it is maintained at a 50 temperature between one approximately optimum for the generation of visible light by radiations and electrons impinging on said phosphor and one only higher to avoid undesirably large envelope size, means electrically connecting said coating to said source, said source when operated producing visible radiations amounting to a substantial portion of the total visible radiations produced by 55 said source and said phosphor, whereby the visible light from said source is augmented and the color thereof modified by the light generated by said phosphor.

60

65

References Cited in the file of this patent  
UNITED STATES PATENTS

|           |                 |                |
|-----------|-----------------|----------------|
| 1,275,890 | Flannery et al. | Aug. 13, 1918  |
| 2,177,705 | Friederich      | Oct. 31, 1939  |
| 2,654,042 | Clarke et al.   | Sept. 29, 1953 |